

Aug. 22, 1933.

R. CLAVER

1,923,189

METHOD FOR LOADING ARTIFICIAL SILK CONTAINING FABRICS

Filed Aug. 23, 1928



Inventor:

René Clavel  
By Emil Bonneycke  
Attorney

## UNITED STATES PATENT OFFICE

1,923,189

METHOD FOR LOADING ARTIFICIAL SILK  
CONTAINING FABRICS

René Clavel, Basel, Switzerland

Application August 23, 1928, Serial No. 301,495,  
and in Switzerland August 23, 1927

4 Claims. (Cl. 8—13)

This invention relates to a process for loading fabrics consisting of or containing artificial silk with metallic compounds and consists in moving the fabric continuously forward and during this movement bringing it into successive contact with solutions of all or part of the substances or mixtures of substances necessary for loading the silk. The operation is preferably carried out by the fabric being passed through a series of baths arranged in succession which, when it is a question of loading with tin phosphate silicate, contain in succession the stannic-chloride, alkali phosphate and silicate solutions. It is not necessary for all the loading agents to act successively on the continuously moving fabric. Thus, for the example, the tin-phosphate silicate loading, only the stannic chloride and the alkali phosphate may be allowed to act on the moving silk fabric and the silicate is then brought into contact with the fabric in the manner hitherto usual, without the fabric being moved forward. When it is a question of producing a lustrous artificial silk it is advisable to treat the fabric with solutions of acids and acid salts before being immersed in the solution of metallic salts or to add acids or acid salts to the metallic salt bath. If, on the other hand, is a question of a matt or dull lustre loading, the treatment with metallic salt in the presence of acids may be eliminated.

It is advisable to squeeze the fabric out on transference from one bath to the next and to lead the loading liquid which is squeezed out back into the previous bath in order to avoid losses in loading agents and any eventual errors in the loading. This squeezing operation is advisable particularly before the artificial silk enters the metallic salt bath, the phosphate bath and the sodium silicate bath which may also be added if necessary and particularly powerful in these cases. The fabric treated with one loading substance may be allowed to remain in contact with the air for a long period before the second loading material acts on the fabric so that the periods of action of the individual liquids on the continuously moving silk fabric shall not be too short. This is preferably effected by the portion of fabric treated with one substance being allowed to remain stationary for a period adjusted as desired before it passes into the bath containing another agent without, however, interrupting the general process and the movement of the remaining portion of fabric. It may be advisable to heat the fabric or to keep it warm during this rest period particularly in the case of treatment with sodium silicate.

A thoroughly satisfactory and unexceptionable

loading of the artificial silk fabric can be obtained in a very short time and with continuous operation by working according to the invention by allowing the individual loading agents to act in succession on the continuously moving artificial silk fabric. A relatively long period has hitherto been necessary for this purpose and continuous operation could not be employed. The degree of loading can also be regulated when working according to the invention by allowing the textile material to pass several times through, for example, the tin and phosphate baths according to the invention; the fabric is preferably well washed between the separate passages. It is also advisable to wash the fabric thoroughly before transferring it to the sodium silicate solution and before winding it off, which can be carried out very simply without interrupting the continuous operation by allowing the fabric to pass through a vessel supplied with water or to remain stationary without, however, interrupting the movement of the fabric in another part of the apparatus.

The application also discloses an apparatus for carrying out the new process which consists essentially of a series of vessels for containing the liquids used in the treatment arranged in succession, i. e.:—in series one after the other or above one another which are provided with a mechanism for moving the fabric continuously forward from the winding-off drum and to guide it through the vessel. These vessels are preferably provided with guide rollers immersed in the liquid below which the fabric is passed through the liquid. The winding-off tanks are arranged between the individual vessels or between groups of vessels in which the corresponding portions of the fabric are stored up and remain stationary for a short or long period as desired before passing through the next vessel. The movement of the portion of the fabric not located in the winding off tank is however not interrupted thereby. The winding off tanks must be constructed so that the artificial silk fabric can enter and emerge therefrom without any hindrance. Those tanks which are open at the top and preferably flat are therefore suitable. In a particularly suitable form of construction these winding off tanks consist of two relatively inclined faces arranged between the individual vessels so that the divergence of the angle formed by the two faces is in the direction of the succeeding vessel. The winding off tanks can be mounted in closed housings in order to be able to heat material or to keep it warm which is par-

ticularly the case when the vessel preceding the corresponding winding off tank contains the sodium silicate solution. It is advisable to provide squeezing means between the individual vessels, particularly before the first vessel for the solution of metallic salt, phosphate solution and silicate solution in order to be able to express the liquid. The washing troughs supplied with washing liquid are attached to the vessel containing the phosphate and, if necessary, to the last vessel containing the sodium silicate and are provided with mechanism guiding the fabric in the trough in several convolutions, for example, a plurality of rollers. The washing troughs may, also, however, be supplied with a mechanism which causes the fabric to rest in the washing trough similarly as in the winding-off tanks without interrupting the movement of the remainder of the fabric thereby. In order to be able to regulate the lengths of the individual periods of rest as simply as possible, it is advisable to attach a so-called "run" to the fabric. Thus, the first run, which may consist for example of a strip of artificial silk is first passed through the machine and the lengths of the first run corresponding to the desired periods of rest are placed in the winding-off tanks and, if necessary, in the washing troughs.

One form of construction of an apparatus suitable for carrying out the new process is shown diagrammatically in the drawing in the form used when it is a question of producing a tin-phosphate-silicate loading in which it is not intended that the artificial silk shall lose its lustre.

The fabric 2 is led from the winding-off drum 1 through a vessel 3 below rollers 4, 5, containing a 10% solution of mono-chlor-acetic acid; after emerging from this vessel the fabric passes through a pair of rollers 6, arranged above and directly behind the vessel, 3, a mechanism, 7, regulating the draw-off and into a tank 8 in which enough artificial silk fabric is allowed to collect to give the necessary period of rest. The silk is then conveyed from this winding-off tank 8 which consists of two relatively inclined plates 9 and 10, preferably fitted with glass, the angle of divergence of which is directed towards the next vessel 11, over a roller 12, and below rollers 13, 14, through water in a vessel, 11, in order to remove excess free acid. From the vessel 11, the artificial silk passes through a squeezing device 15 into the vessel 16 which contains a solution of stannic chloride of specific gravity 35° Bé. and also provided with guide rollers 17 and 18. From this vessel 16 the artificial silk then passes over a pair of rollers 6a, a winding-off device 19 in and through a winding-off tank 20 of the same construction as the tank 8. Enough artificial silk is again collected at this point to give the desired period of rest. The artificial silk is then led over a roller 21 through a second vessel 22, provided with guide rollers, 23 and 24, also containing a 35° Bé. stannic chloride solution, to be collected again after emerging from this vessel, 22, in a winding-off tank 25 in which the desired period of rest is obtained.

The fabric 2, then passes over a stretcher 26 of the usual construction in which the fabric is finally again widened, through a squeezer, 27 and into a vessel 28, containing a 10% solution of mono-sodium-di-hydrogen-phosphate and also provided with guide rollers 29, 30. The fabric again passes from this vessel 28 into a winding-off mechanism 31 in which sufficient artificial silk is collected to give the necessary length for the

desired period of action of the mono-sodium-di hydrogen-phosphate. The artificial silk is then again passed through a stretcher 32 into a vessel 33 provided with one or more guide rollers 34 and containing di-sodium-mono-hydrogen-phosphate with the addition of a small quantity of sodium carbonate. A washing trough 35 supplied with running water and having a plurality of guide rollers, 36, in order to lead the fabric through the washing trough in several convolutions follows this vessel.

The continuous loading process can be interrupted at this point and the silicate treatment carried out in the manner hitherto usual without continuous movement of the artificial silk fabric. Further additional vessels, winding-off devices and squeezers similar to the devices 15-31 can be inserted after the winding-off tank 31 before the vessel 33, in order to allow further passage through the tin and phosphate before treatment with silicate. The fabric from the winding-off tank 31 may also be again passed through the squeezer 15 and the devices succeeding thereto, one or more times in order to make several passages through the tin and phosphate baths.

In this connection it is, however, advisable to wash the artificial silk before each fresh passage for example, in washing troughs such as 35. The vessel, 33, containing the phosphate solution having an alkaline reaction through which the artificial silk passes before the treatment with the silicate can be eliminated. In this case it is advisable to add di-sodium-mono-hydrogen-phosphate and some sodium carbonate to the washing water in the trough 35.

The artificial silk fabric emerging from the washing trough 35 is then again led through a stretcher 37 and a squeezer 38 into a vessel provided with guide rollers 40 and 41 and containing a solution of sodium-silicate of specific gravity of at least 1° Bé. and with 2 grammes soap per litre at 60° C. From this vessel 39 the fabric passes over a roller 42 into the vessel which contains a solution of sodium silicate specific gravity of at least 1° Bé. at 60° without the addition of any soap and is also provided with guide rollers 44 and 45. From the vessel 43, the fabric 2 passes into a winding-mechanism 46, entirely enclosed by a casing so as to prevent the temperature of the fat dropping below 50° C., in this chamber, which is also heated. The vessel 48, following this winding-off tank 46 again contains a solution of sodium silicate of at least 1° Bé. at 60° C. and is provided with guide rollers 49 to 50. A winding-off mechanism 51 with a housing 52, in order to prevent the temperature of the artificial silk dropping below 50° C. follows this vessel 48. The artificial silk is then heavily loaded and passes through a stretcher 53 into a washing trough provided with guide rollers and supplied with soft water. From this washing trough the fabric 2, passes over a roller 56, through a winding mechanism 57 and on to a table 58, where it is piled up. A winding mechanism may also be provided instead of this table 58.

The arrangement described as an example of construction may be modified very extensively without departing from the scope of the invention. Thus, for example, several vessels containing the same liquid may be arranged after another or above one another. A number of these vessels can be suitably arranged according to the speed with which the artificial silk is

be loaded and according to the degree of loading to be produced. Further winding-off devices which insure the material resting for a period before entering the fresh bath may be omitted.

5 In this case, other devices must be provided which render possible the resting of the artificial silk in the individual vessels for containing the liquids used for the treatment or provision must be made that the artificial silk is led through

10 the separate baths at only a very low velocity. The vessels containing the liquids can be provided with heating devices for example, heating pipes in order to be able to adjust the temperature to any predetermined value. The whole apparatus

15 is preferably driven by a single motor with suitable connecting and transmission gears.

By artificial silk I mean any kind of synthetic textile material having the appearance of natural silk and consisting mainly of cellulose derivatives.

20 I claim:

1. A method for loading artificial silk containing fabrics in which the fabric to be loaded is passed continuously through baths containing in 25 succession a solution of an organic acid, tin tetrachloride solution, and alkali-metal phosphates.

2. A method of loading artificial silk contain-

ing fabrics, in which the fabric to be loaded is moved continuously forward, which comprises moving the fabric successively through an acid bath and squeezing out the fabric, moving the fabric through a metal salt bath and squeezing out the fabric, and then moving the fabric through a bath of alkali phosphate.

3. A method of loading artificial silk containing fabrics, in which the fabric to be loaded is moved continuously forward, which comprises moving the fabric successively through an acid bath and squeezing out the fabric, moving the fabric through a metal salt bath and squeezing out the fabric, and then moving the fabric through a bath of mono-sodium-di-hydrogen-phosphate.

4. A method of loading artificial silk containing fabrics, in which the fabric to be loaded is moved continuously forward, which comprises moving the fabric successively through an acid bath and squeezing out the fabric, moving the fabric through a metal salt bath and squeezing out the fabric, and then moving the fabric through a bath of mono-sodium-di-hydrogen-phosphate and then moving the fabric through 100 a bath of di-sodium-di-hydrogen-phosphate.

RENÉ CLAVEL.

30

105

35

110

40.

115

45

120

50

125

55

130

60

135

65

140

70

145

75

150